

## UNITED STATES PATENT OFFICE

2,157,654

## MANUFACTURE OF ARTICLES FROM STEEL ALLOYS

Friedrich Karl Naumann, Essen, Germany, assignor to Fried. Krupp Aktiengesellschaft, Essen-on-the-Ruhr, Germany

No Drawing. Original application March 3, 1934, Serial No. 713,926. Divided and this application September 13, 1937, Serial No. 163,619. In Germany March 20, 1933.

## 8 Claims. (Cl. 75—126)

This invention relates to the manufacture of articles that by their nature are subjected in use to, and must withstand the attack of, hydrogen at high hydrogen partial pressures and high temperatures such as apparatus and parts thereof which are used in the destructive hydrogenation of oil and coal, or in the synthesis of ammonia, and with which hydrogen or mixtures of gases containing hydrogen come into contact at high temperatures and pressures.

In my co-pending application for Letters Patent, filed November 22, 1933, Serial Number 699,300, I propose to manufacture articles of this class from steel alloys which contain titanium and if desired one or more of the elements silicon, manganese, nickel, cobalt, chromium, tungsten, molybdenum and vanadium, the steel alloys suitably containing up to 1% carbon, up to 5% titanium, and if desired up to 30% of one or more of the elements silicon, manganese, nickel, cobalt, chromium, tungsten, molybdenum and vanadium.

In my co-pending application for Letters Patent, filed March 3, 1934, Serial Number 713,926, of which the present application is a division I have shown that besides titanium also the other elements of group IV of the periodic table, as far as they form carbides in the steel, viz., zirconium and thorium, have the property of rendering steel resistant to the attack of gases that attack and remove carbon, such for instance as the attack of hydrogen at high temperatures and pressures.

According to the present invention use is made for the manufacture of the articles in question of steel alloys which contain an effective amount of one or more elements selected from the group zirconium and thorium and one or more of elements improving the creep strength of the alloy, viz., chromium tungsten molybdenum and vanadium.

Preferably the content of the elements zirconium and thorium amounts to not over 5% and the carbon content to not more than 1%, while the total content of the elements chromium, tungsten, molybdenum and vanadium may amount about up to 30%. In general, however, a total content of not more than 15% of these elements is found desirable. The balance of the alloy consists substantially of iron with the normal contents of Mn and Si. The latter content, however, may amount also up to 1.5%.

The addition of one or more of the elements Cr, W, Mo and V has for its object to improve the creep strength of the steel alloys, since this

property is of great importance for the apparatus which operate at elevated temperatures.

The steel alloys which besides the carbide-forming element of group IV contain further additions of elements, improving the creep strength of the alloys, show a resistance to carbon-removing gases which far exceeds the effect of these additional elements, as the following test shows:

From two steel alloys, A, B of the following composition

| Steel | Percent C | Percent Si | Percent Mn | Percent Cr | Percent Zr | Percent Mo |
|-------|-----------|------------|------------|------------|------------|------------|
| A     | 0.10      | 1.43       | 0.48       | 1.22       | 0.95       | ...        |
| B     | 0.10      | 1.07       | 0.58       | 1.19       | ...        | 0.58       |

tensile test pieces were prepared and likewise heated 100 hours at 600° C. in hydrogen under pressure of 300 at. The test pieces treated in this manner showed the following data of strength:

| Steel | Yield point, kg/mm. <sup>2</sup> | Tensile strength, kg/mm. <sup>2</sup> | Extension 5×d | Reduction in area | Hardness |
|-------|----------------------------------|---------------------------------------|---------------|-------------------|----------|
| Aa    | 44                               | 53.8                                  | 24.5          | 59                | 169      |
| ab    | 42                               | 51.2                                  | 23.0          | 57                | 162      |
| Ba    | 41                               | 53.4                                  | 33.3          | 78                | 149      |
| bc    | 26                               | 32.7                                  | 13.7          | 16                | 110      |

wherein by a is marked the state when supplied and by b the state after the test.

This table shows that the steel marked A remained practically unaltered, whilst the steel B suffered a considerable deterioration of its properties of strength.

Steel alloys have been found particularly suitable for the purposes according to the invention, which contain about up to 0.4% carbon, up to 2% zirconium, up to 3% molybdenum or vanadium, separate or mixed and if required up to 10% chromium.

I claim:

1. Articles which in their normal use are subjected to the attack of hydrogen at high hydrogen partial pressures and high temperatures, said articles being composed of a steel alloy consisting of carbon not over 1%; up to 30% of material from the group consisting of chromium, molybdenum, tungsten, and vanadium; and an effective amount not over 5% of material from the group consisting of zirconium and thorium; the remainder substantially iron with silicon not over

5

10

15

20

25

30

35

40

50

55

about 1.5% and a manganese content within the usual range for low alloy steels.

2. Hydrogenating apparatus having its parts which are subjected to the attack of hydrogen at high pressure and temperature, composed of a steel alloy consisting of carbon not over 1%; up to 30% of material from the group consisting of chromium, molybdenum, tungsten, and vanadium; an effective amount not over 5% of material from the group consisting of zirconium and thorium; the remainder substantially iron with silicon not over about 1.5% and a manganese content within the usual range for low alloy steels.

3. Articles which in their normal use are subjected to the attack of hydrogen at high hydrogen partial pressures and high temperatures, said articles being composed of a steel alloy consisting of carbon not over 1%; up to 15% of material from the group consisting of chromium, molybdenum, tungsten, and vanadium; an effective amount not over 5% of material from the group consisting of zirconium and thorium; the remainder substantially iron with silicon not over about 1.5% and a manganese content within the usual range for low alloy steels.

4. Hydrogenating apparatus having its parts which are subjected to the attack of hydrogen at high pressure and temperature composed of a steel alloy consisting of carbon not over 1%; up to 15% of material from the group consisting of chromium, molybdenum, tungsten, and vanadium; an effective amount not over 5% of material from the group consisting of zirconium and thorium; the remainder substantially iron with silicon not over about 1.5% and a manganese content within the usual range for low alloy steels.

5. Articles which in their normal use are subjected to the attack of hydrogen at high hydrogen partial pressures and high temperatures, said articles being composed of a steel alloy consisting of carbon not over 0.4%; up to 3% of molyb-

denum; an effective amount not over 2% material from the group consisting of zirconium and thorium; the remainder substantially iron with silicon not over about 1.5% and a manganese content within the usual range for low alloy 5 steels.

6. Articles which in their normal use are subjected to the attack of hydrogen at high hydrogen partial pressures and high temperatures, said articles being composed of a steel alloy consisting of carbon not over 0.4%, up to 3% of molybdenum; up to 10% chromium; an effective amount not over 2% of material from the group consisting of zirconium and thorium; the remainder substantially iron with silicon not over about 1.5% and a manganese content within the usual range for low alloy 10 steels.

7. A process which comprises subjecting a material to be hydrogenated to the influence of hydrogen at high hydrogen partial pressure and high temperature in a container composed of a steel alloy containing carbon not over 1%; up to 30% of material of the group consisting of chromium, molybdenum, tungsten and vanadium; and an effective amount not over 5% of material 20 from the group consisting of zirconium and thorium; the remainder substantially iron with silicon not over about 1.5% and a manganese content within the usual range for low alloy steels.

8. A process which comprises subjecting a material to be hydrogenated to the influence of hydrogen at high hydrogen partial pressure and high temperature in a container composed of a steel alloy containing carbon not over 0.4%; up to 3% of molybdenum; up to 10% of chromium; 30 an effective amount not over 2% of material from the group consisting of zirconium and thorium; the remainder substantially iron with silicon not over about 1.5% and a manganese content within the usual range for low alloy steels.

FRIEDRICH KARL NAUMANN. 40